

# UNITED STATES PATENT OFFICE.

OSCAR OSTERSETZER, OF SAGAN, GERMANY.

## PRINTING COTTON FABRICS.

SPECIFICATION forming part of Letters Patent No. 501,156, dated July 11, 1893.

Application filed February 17, 1893. Serial No. 462,762. (No specimens.)

*To all whom it may concern:*

Be it known that I, OSCAR OSTERSETZER, a subject of the Emperor of Austria-Hungary, and a resident of Sagan, Austria-Hungary, 5 have invented certain new and useful Improvements in Methods of Discharging Red and other Azo Colors on Direct-Dyeing Cotton Dye-Stuffs, of which the following is a specification.

10 On account of the brilliancy of red-azodyes it has for a long time been tried to print the same with a discharge on bottoms dyed with so-called aniline colors, but this has hitherto not been possible, because all azodyes are destroyed by the means which are used for discharging the bottom.

15 The object of this invention is to overcome this difficulty by developing the red on the fiber. Thus not only red in its various shades 20 but also yellow, orange, brown and other shades can be produced.

This invention may be carried out as follows: Recently a series of direct dyeing cotton-dyes have been found, which can be diazotized on the fiber and developed to new dyestuffs, which latter not only differ in shade 25 from the original dyeing, but also show a greater resistance to the actions of light, alkalies and acids. These dyestuffs belong to two different groups, the first one of which is characterized by the dyestuff, named primuline; (thiochromogene, polychromine,) the second one by diamineblack (diamineblueblack, Nyanza or tabora-black, diazurine, diazochromine). The first one of these groups is distinguished from the second one by its resistance 30 against reducing agents. If therefore a printing paste which contains a dyestuff of the first group and a reducing agent is applied to a tissue dyed with a dyestuff of the second group, this latter after steaming will disappear on the printed spots while simultaneously the first one is fixed on these spots, and a pattern can thus be produced, which however 35 does not possess the usually desired fastness to washing. Whereas however such dyestuffs are selected which by the well known method may be further diazotized and developed to shades fast to washing, it results that 40 by passing the goods through nitrite of soda

and then through a bath containing a suitable phenole or amine, both the printed and the bottom colors can be perfectly fixed.

As developers I particularly name the following: phenole, resorcine, beta-naphthol, 55 Schaeffer-acid, ethyle-beta-naphthylamine, phenylenediamine.

On bottoms dyed as above mentioned I obtain by developing with betanaphthol—turkey red print on blue ground; by developing 60 with Schaeffer acid—scarlet print on blue ground; by developing with ethyle betanaphthylamine—claret red print on blue ground. By developing diamine black I obtain with phenylenediamine—red print on black 65 ground; resorcine—orange print on black ground.

I give the following examples:

*Example I.*—Turkey red shade on dark-blue by means of betanaphthol. I dye for instance with five per cent. diamine blueblack E with the usual addition of glaubersalt and soda and then I print thereon the following printing paste: five hundred grains primuline, one thousand grains dextrine, two thousand grains water, twelve hundred grains zinc-dust, nine hundred grains bisulphite 70 75 30°, one hundred and twenty grains glycerine, eighty grains ammonia. Then I steam during one hour. After steaming, in order 80 to remove the zinc-dust, which would impair the formation of the new azodye, the goods are passed through diluted muriatic acid and then diazotized in a cold solution containing three hundred grains nitrite of 85 soda and one liter muriatic acid of 21° Baumé to two hundred liters water. Then the goods are entered in a bath containing four hundred grains of betanaphthol dissolved in one hundred and ten grains caustic soda and one 90 hundred liters water. Instantly the shade of the bottom turns into a darkblue and the print into red.

*Example II.*—In order to produce red print on black ground, I dye with five per cent. diamine black and print as stated in Example I, then diazotize as above described and develop in a solution of two hundred and sixty grains phenylenediamine in two hundred liters water.

The thus produced patterns are of great fastness to washing and acids, but less fast to light than the known turkey red-indigo fabrics, against which my method has the advantage of cheapness.

What I claim as new, and desire to secure by Letters Patent, is—

The process of printing cotton fabrics which are dyed with a diazotizable azo dye-stuff, such as diamine black, by means of a printing color consisting of a diazotizable but not reducible dye-stuff such as primuline, and a reducing agent, and of developing the printed

design by steaming, passing through an acidulated bath of nitrite of soda and passing <sup>15</sup> through a second bath which contains a phenol or an amine, substantially as herein described.

In testimony that I claim the foregoing as my invention I have signed my name, in presence of two witnesses, this 22d day of January, 1893.

OSCAR OSTERSETZER.

Witnesses:

ADOLF DEMUTH,  
OTTO GOLDSCHMIEDT.